

# UNITED STATES PATENT OFFICE.

JOHN G. HOMAN, OF STEUBENVILLE, OHIO, ASSIGNOR, BY MESNE ASSIGNMENTS, TO  
WILLIAM H. KELLER, OF NORTON, VIRGINIA.

## ALLOY.

1,352,367.

Specification of Letters Patent.

Patented Sept. 7, 1920.

No Drawing.

Application filed January 3, 1920. Serial No. 349,238.

To all whom it may concern:

Be it known that I, JOHN G. HOMAN, a citizen of the United States, and a resident of Steubenville, in the county of Jefferson 5 and State of Ohio, have invented a new and useful Improvements in Alloys; and I do hereby declare the following to be a full, clear, and exact description thereof.

My invention relates to alloys and has 10 special reference to an iron alloy for use in the production of sheets or plates for punched or stamped resistance grids, such as is shown and described in United States Letters Patent granted to William H. Keller, 15 No. 1,184,706, dated May 23, 1916, and No. 1,240,457, dated September 18, 1917.

In the practice of producing resistance grids, such as is done under the stamping or 20 punching process from sheets or plates, it was contemplated by the above mentioned 25 patents to use only steel for such purpose, and it has been found that certain steels or alloys have a higher resistance than ordinary steel and from this point of view would be desirable material, but it has also been found in practice that a steel containing say five (5%) per cent. of silicon cannot 30 be satisfactorily punched into such grids of desirable thickness without excessive breakage.

The object of my invention is to provide an iron alloy which will overcome such objections and give the desired resistance for such grids by producing a punchable 35 material of electrical resistance superior to iron.

To these ends my invention consists, generally stated, in the novel form of an alloy as hereinafter more specifically set forth 40 and described and particularly pointed out in the claims.

To enable others skilled in the art to which my invention appertains to construct and use my improved alloy, I will describe 45 the same more fully.

It is known that iron when alloyed with silicon could be made into a rather inexpensive alloy but for its brittleness. On the other hand, those alloys of iron formed from 50 elements of even numbered series of the periodic system produced alloys of mechanical strength, although it is known, however, that alloys of even series were objectionable as regards magnetic value.

An alloy of iron and silicon is produced 55 in the ordinary way by adding sufficient silicon to make the resistance desired. If a relatively high specific resistance is desired it is aimed to get—say five (5%) per cent. silicon, and if a medium resistance is 60 desired it is aimed to get say two (2%) per cent. silicon. To this material, as thus prepared, manganese to the extent needed is added to secure mechanical working, and the two (2%) per cent. silicon alloy will not 65 require more than .20% manganese, while the five (5%) per cent. silicon alloy may require one (1%) per cent. to get results. However, it is not desired to be limited to manganese to gain such results as it has been 70 found that carbon may be a valuable adjunct and the use of it valuable in making grid material, so that the addition of .10% to .25% carbon in some alloys is advantageous. 75

Various other changes and additions and eliminations of materials may be resorted to, without departing from the spirit of the invention or sacrificing any of its advantages, and obviously the normal content of 80 other elements exist, as impurities in steel, and are not considered as part of this invention.

What I claim as my invention and desire to secure by Letters Patent is: 85

1. An alloy of iron and silicon having an electrical resistance superior to iron and of punchable quality, consisting of iron, silicon 1% to 6% and manganese .20% to 1%, the relation of the silicon and manganese being such, as one of them is increased or diminished, the other is also more or less increased or diminished. 90

2. An alloy of iron and silicon having an electric resistance superior to iron and of 95 punchable quality, and consisting of iron, silicon 1% to 6%, carbon .10% to .25% and manganese .20% to 1%, the relation of the silicon and manganese being such, as one of them is increased or diminished, the other is also more or less increased or diminished. 100

3. In a resistance grid, rheostat or similar appliance, an alloy of iron and silicon having an electrical resistance superior to iron 105 and of punchable quality, consisting of iron, silicon 1% to 6% and manganese .20% to 1%, the relation of the silicon and man-

ganese being such, as one of them is increased or diminished, the other is also more or less increased or diminished.

4. In a resistance grid, rheostat or other similar appliance, an alloy of iron and silicon having an electrical resistance superior to iron and of punchable quality, consisting of iron, silicon 1% to 6%, carbon .10% to .25% and manganese .20% to 1%, the re-

lation of the silicon and manganese being 10 such, as one of them is increased or diminished, the other is also more or less increased or diminished.

In testimony whereof I, the said JOHN G. HOMAN, have hereunto set my hand.

JOHN G. HOMAN.

Witness:

J. M. GEOGHEGAN.